

## UNITED STATES PATENT OFFICE

2,171,475

## METHOD OF FIXING CLOTH FINISHES

Hilton Ira Jones and Llewellyn Jones,  
Wilmette, Ill.No Drawing. Application December 8, 1936,  
Serial No. 114,832

## 1 Claim. (Cl. 91—68)

This invention relates to improvements in the finishing of textiles, and its objects are as follows:

First, to so treat cloth, or equivalent textile fabrics, in such a manner as to make it permanently retain a desired applied finish.

Second, to so treat a finishing substance for cloth and similar textile fabrics, as to render its adhesion to the cloth permanent.

10 Third, to provide a starch having the characteristic that when a piece of cloth is starched with it, the cloth may be washed and ironed indefinitely without losing its stiffness or finish.

Other objects and advantages will appear in 15 the following specification to which reference is made for the various steps by which the results of the process are accomplished.

Everyone knows that the prevailing modes of 20 finishing cloth are lacking in the quality of durability, certainly in so far as the well known steps of starching and filling are concerned. A starched piece of goods, for example, a collar, retains its finish only between laundering. Piece goods are commonly sold with a filling, 25 especially the cheaper varieties of goods, which imparts a certain degree of body and stiffness while new but which is lost with the first washing.

As indicated in the foregoing statements of the 30 objects of the invention, the improved method provides a means of permanently affixing to fabrics a desired finishing element, for example, starch, so that said finishing element will not be removed either by laundering or dry cleaning. 35 The manner in which this is accomplished is now set out. Provision is made, in the preferred practice of the method, for two baths, herein designated baths A and B. Bath A may consist, for example, of:

|               | Percent  |
|---------------|----------|
| Corn starch   | 1 to 3   |
| Stearate soap | 2½ to 7½ |
| Water to make | 100      |

40 These ingredients are mixed cold and then brought to a boil to cook the starch.

Bath B will consist of a solution of rare earth acetates, formates or furoates of from 1 to 5 per cent concentration. The rare earth acetates, 45 formates or furoates intended to be used are such as are disclosed in the patents to Hilton Ira Jones, No. 1,688,717 of Oct. 23, 1928; No. 1,799,047 of Mar. 31, 1931; and 1,921,926 of Aug. 8, 1933.

50 Among the salts of the rare earth metals which may be employed we refer particularly to the

acetates, formates, or furoates of cerium, thorium, lanthanum, or the radio-active metals, such as uranium, or a combination of any of these, or of one or more of these with aluminum, tin or other metallic salts. The exact concentration of the solution is not of great importance, as explained below.

5 The textile, preferably in the bolt, is passed through bath A which is preferably kept warm, but not boiling. Bath A is supplemented with a 10 suitable arrangement to insure the penetration of the textile by the solution. This arrangement may comprise any kind of guard or rolls that will keep the textile submerged. As the textile passes through the solution in bath A 15 it is directed through a set of squeeze rolls which remove the excess solution.

Naturally the adjustment of these rolls will 20 determine the pressure and, consequently, the amount of the solution that is allowed to remain in the textile as it passes on to bath B. The equipment in bath B is similar to that in bath A, the sole purpose being to thoroughly impregnate the textile and so precipitate the soap which carries the starch.

25 As the textile passes from bath B it is wrung out again by a duplicate set of squeeze rolls so as to remove the excess. In practice the second set of rolls is tightened considerably so that but a small excess of B bath solution remains in the 30 goods. As the impregnation of the textile continues, the concentration of the solution in bath B becomes continuously less and must be strengthened from time to time in order to bring it up to its original condition by the addition of 35 more of the rare earth salts, for example, cerium acetate as suggested in Patent No. 1,688,717. After the goods have passed the squeezing operation at bath B, they are dried over steam-heated drums or by any equivalent device, and this 40 either with or without first rinsing them.

It has been discovered that by the practice of the foregoing method it is possible to permanently affix to cloth or equivalent textile fabrics, 45 many substances, for instance starch, which will otherwise readily wash out either by laundering or dry cleaning. The effect of first subjecting the goods to the stearate or other soap in bath A, wringing the goods out and then subjecting it to bath B, is that a rare earth stearate is 50 precipitated which encloses or entangles the starch, combining it with the threads of the goods in such a way that when the goods is rinsed, dried and ironed, the starch cannot be removed by washing or dry cleaning. The re- 55

- sulting finish withstands laundering to an unusual degree. In actual experimentation and demonstration, textiles treated according to the foregoing method have been boiled in a 5 per cent solution of a commercially known type of laundry flakes for thirty minutes with constant agitating then rinsed and ironed, the whole operation having been repeated for more than one hundred times with no effect upon the finish.
- 5 Other similarly treated pieces were laundered and ironed in a commercial laundry without effect upon the finish, then they were further continuously washed by the same laundry for a period of one week, then finally rinsed and 10 ironed, after which the finish of the cloth still seemed unaffected. In this way, cottons, for example, may be washed and ironed indefinitely and will remain as stiffened and finished as they were in the beginning.
- 15 By this same method many other substances may be permanently affixed to textiles. Among these bentonite is one. This substance has the quality of delustering the goods. Other substances may be similarly affixed, for instance, 20 precipitated chalk or commercial fire-repellant salts for fire-proofing, as well as all sorts of waxes and gums (as an emulsion in the A bath) for increasing the sheen or otherwise modifying the finish. It is also contemplated to employ 25 many other metallic salts in the B bath along with the rare earths, for example, aluminum acetate or formate, and in this way the stearates formed by precipitation are thus rendered permanent and not removed by washing or dry 30 cleaning as they would otherwise be.
- 35 While in practice the stearate soaps are used (bath A) because they are cheaper than others and just as satisfactory, it must be understood that the oleates, palmitates and all other similar 35 soaps may be used.
- 40 A further modification of the method which

has been found to be valuable is to use along with the soap solution in the A bath (in place of the starch, bentonite, or similar ingredients) soluble proteins which are also precipitated by the rare earths in bath B. Among the best of 5 these proteins is the so-called alpha protein as extracted from soy beans. The same or any equally satisfactory soluble protein may be extracted from soy bean flour by boiling said flour with water and then filtering it. The filtrate 10 contains the soluble proteins. These proteins used in this way will thus be precipitated along with the stearates. They provide excellent finishing and stiffening agents and may be used along with or in place of the starch.

15

In many cases it is possible to incorporate the soap and starch or other ingredient directly in the dye bath, and thus avoid the necessity of a second bath for the finishing. Thus it will be understood that the main purpose of the method 20 is to permanently affix to fabrics such finishing substances as starch, bentonite, etc., for the stiffening, filling, delustering, fireproofing, etc., so that these treatments are made permanent 25 and are not removed by laundering or dry cleaning. The rare earth, and other metallic soaps, as above mentioned, are used as carrying or affixing agents for the starch, bentonite, etc.

25

We claim:

The method of treating textiles to affix a 30 finish, consisting of immersing the textile in a bath of 1 to 3 percent cornstarch, 2½ to 7½ percent stearate soap and approximately 95 percent water, wringing the textile to remove the surplus bath solution, again immersing the textile 35 in a bath of rare earth acetates of 1 to 5 percent concentration, wringing the textile to remove the surplus solution of the second bath, and drying the wrung textile.

35

HILTON IRA JONES. 40  
LLEWELLYN JONES.